

# United States Patent

[11] 3,621,430

[72] Inventor **Yohel Shimizu**  
Nishinomiya, Japan  
[21] Appl. No. **22,138**  
[22] Filed **Apr. 2, 1970**  
[45] Patented **Nov. 16, 1971**  
[73] Assignee **Sanyo Electric Co., Ltd.**  
Moriguchi-shi, Japan  
[32] Priority **Oct. 28, 1967**  
[33] **Japan**  
[31] **42/69529**  
Continuation of application Ser. No.  
**771,297, Oct. 28, 1968, now abandoned.**

[54] **FLYBACK TRANSFORMER COIL FOR  
TELEVISION RECEIVER**  
3 Claims, 2 Drawing Figs.  
[52] U.S. Cl..... **336/205,**  
336/206, 336/96  
[51] Int. Cl..... **H01j 27/30**

[50] **Field of Search**..... 336/96,  
205, 206; 260/94.7

[56] **References Cited**  
UNITED STATES PATENTS

|           |         |                 |           |
|-----------|---------|-----------------|-----------|
| 2,295,958 | 8/1942  | Lutz .....      | 336/205 X |
| 2,464,568 | 3/1949  | Flynn .....     | 336/205 X |
| 3,225,269 | 12/1965 | Worcester ..... | 336/205 X |
| 3,235,825 | 2/1966  | Davis.....      | 336/205   |

*Primary Examiner—E. A. Goldberg*

**ABSTRACT:** Flyback transformer coil for television receiver comprises surface-insulated wire windings having a plurality of wire layers, a plurality of layers of insulating material thereby to separate adjacent layers of wound wires, and an assembly of the windings and interpositioned insulating material being impregnated with a liquid heat-setting 1-2 polybutadiene resin having a lower dielectric loss at both low and high temperatures, for example 20°—150° C., and heated and hardened, thereby to deposit a hardened layer of the resin in all the layers of the coil assembly.

The present coil has a good water, moisture and burning resistances and good insulating efficiency.



PATENTED NOV 16 1971

3,621,430

FIG. 1



FIG. 2



INVENTOR  
YOHEI SHIMIZU

BY Darby & Darby

ATTORNEY

**FLYBACK TRANSFORMER COIL FOR TELEVISION  
RECEIVER**

This is a continuation of Ser. No. 771,297 filed Oct. 28, 1968 now abandoned.

The present invention relates to a coil for flyback transformer of television receiver, and more particularly to an improved coil for flyback transformer having a good water and moisture resistance, good burning resistance and good insulating efficiency.

A flyback transformer is employed in a television receiver to couple the horizontal sweep signal from the horizontal output stage to the deflection yoke and to develop the high voltage necessary for operation of the cathode-ray tube. Such transformers also conveniently perform ancillary functions such as developing horizontal flyback pulses for application to the AGC keyer and developing blanking pulses for application to the cathode-ray tube. The flyback transformer is thus a high-voltage, high-energy device and must be carefully designed to insure compliance with rigid safety standards.

In the prior art flyback transformer now employed throughout the industry, a layer wound coil employing a kraft paper tape or polyethylene terephthalate tape as the insulating material and being impregnated with wax material or heat-setting epoxy resin is used as the secondary coil or high-voltage coil for the flyback transformer.

In the secondary coil impregnated with the wax material, for example, microcrystalline wax, the wax material is melted at an elevated temperature, and thus the wax material starts to flow. This results in an increase in flyback transformer temperature and the insulation of the transformer is deteriorated.

Further, the wax material-impregnated coil tends to burn with an increase in flyback transformer temperature.

It is a practice to place a corona tire, a compound molding, around the outer surface of the secondary or high-voltage coil to prevent corona which would otherwise result in failure of the transformer.

In the wax material-impregnated coil, a high temperature and high pressure are applied to the coil when the corona tire is placed thereon, and as a result the coil tends to be deformed.

In the heat-setting epoxy resin-impregnated coil, the epoxy resin itself has a high dielectric loss at a high temperature, for example 60° or higher, and thus the flyback transformer temperature tends to be raised so that there often occurs burning of the transformer.

An extensive study of the impregnating materials suitable for the flyback transformer coil, the present inventor has succeeded in eliminating all the above-mentioned troubles encountered in the conventional secondary or high voltage coil for the flyback transformer.

The object of the present invention is to provide a coil for the flyback transformer, which has a good water resistance, good moisture resistance, good burning resistance and good insulating efficiency.

The invention together with further objects and advantages will be understood by reference to the accompanying drawings in which:

FIG. 1 is a perspective view, partially in section, of a flyback transformer for a television receiver.

FIG. 2 is a sectional view showing the coil, insulating material and papers in accordance with this invention.

Referring to FIGS. 1 and 2, a coil assembly 1 comprises a primary coil 3 wound on the spool 2 and secondary coil 4 on another spool 5.

The coils comprise surface-insulated wire 6, and a plurality of wire layers 7 separated by layers of insulating material 8. As is conventional, the coil assembly is further equipped with a lead 9 and a cap 10 which transfer the high voltage from the secondary coil to a high-voltage rectifier (not shown). Reference numeral 11 is a corona tire.

According to the present invention, a coil consists of the surface-insulated wire windings 6 in a coil form having a plurality of wire layers 7, a plurality of layers of insulating material 8, adjacent layers of wound wires being separated by a layer

5 of the insulating material, and an assembly of the wirings and interpositioned insulating material being impregnated with a liquid heat-setting 1-2 polybutadiene resin having less dielectric loss at both low and high temperatures, for example, 20°-150° C., and heated and hardened thereby to deposit a hardened layer of said resin in all the layers of the coil assembly.

10 In the present invention, the insulating material includes a paper tape 8 such as a kraft paper tape, polyethylene terephthalate tape and other tapes having a suitable insulating effect.

15 The liquid polybutadiene resin used in the present invention includes atactic 1-2 polybutadiene,  $\alpha$ ,  $\Omega$ -polybutadiene glycol and  $\alpha$ ,  $\Omega$ -polybutadiene carboxylic acid, which are commercially available in trademarks "Nisso-PB," "Nisso-PGB" and "Nisso-PBC" respectively, those being manufactured by Nihon Soda Co., Ltd., Japan. The liquid polybutadiene used in the present invention is a liquid viscous polymer having a number mean molecular weight of 1,000 to 5,000 specific gravity of 0.86 to 0.90 ( $d_4^{15}$ ). The liquid polybutadiene resin itself undergoes cross-linking by auto-oxidation at the ordinary temperature by leaving the liquid polybutadiene resin in a film state in air, and a hardened film is thereby obtained. However, the hardening can be promoted by adding a very small amount of metal salt or peroxide as a catalyst or can be effected in a very short time, for example, 30 min., by heating the resin to 130° to 150° C. The cross-linking of the liquid 20 polybutadiene resin is based on an autoxidation mechanism in the presence of air or oxygen, which is similar to that of such a drying oil as linseed oil. A clear resin having a high hardness can be also obtained by adding a radical polymerization initiator to the liquid polybutadiene resin and heating the added liquid resin to 120° to 140° C. for 20 to 80 minutes.

25 The thus obtained hardened resin has a high mechanical strength, high heat deformation temperature and high insulating efficiency as shown below:

Mechanical properties:

30 Density, g/cm.<sup>2</sup> : 0.94 - 0.97

Hardness (Shore D) : 64 - 75

Bending strength, kg./mm.<sup>2</sup> : 3.0 - 3.5 (ASTM-D-790)

Compression strength, kg./mm.<sup>2</sup> : 7.1 - 8.6 (ASTM-D-695)

Impact strength (Charpy), kg.cm./cm.<sup>2</sup> : 4.5 - 5.2

Hygroscopicity : 0.01 - 0.03% (60° C., 5 hr)

Molding shrinkage : 3.3 - 3.5 % (linear shrinkage)

35 Thermal property

Heat deformation temperature: 200° C. (ASTM-D-648)  
(load: 264 lb/in<sup>2</sup>)

Electrical properties

40 Surface resistivity :  $10^{16}$  -  $10^{17}$   $\Omega$  (ASTM-D-257)

Volume resistivity :  $10^{16}$  -  $10^{17}$   $\Omega$  (ASTM-D-257)

Dielectric constant 30 c./s. : 2.7 (ASTM-D-150) 1 mc./s. : 2.7 (ASTM-D-150)

tan  $\delta$  30 c./s. : 0.002 1 mc./s. : 0.002

45 In the present invention, it is preferable, in view of the productivity, to use a liquid polybutadiene consisting substantially of 1-2 polybutadiene resin and harden the same by heat-setting to shorten the processing time.

50 The present invention is explained hereunder, referring to examples:

**Example 1**

55 A coil was prepared by winding a 0.12  $\Phi$ , polyurethane-insulated wire using a 0.08 mm.-thick kraft paper tape as an interlayer, insulating material. Then, the wound assembly was impregnated with a liquid 1-2 polybutadiene resin, and heated to 135° C. for 3 hours thereby to form a hardened layer of the resin in all the layer of the coil assembly. Then, a proper corona tire was placed on the surface of the deposited resin layer in the ordinary manner thereby to prepare a high-voltage coil.

3  
Example 2

A high voltage coil was prepared by winding a 0.12 Φ polyurethane-nylon2insulated wire using a 0.8 mm.-thick polyethylene terephthalate tape as an interlayer insulating material. Then, the wound assembly was impregnated with a liquid 1-2 polybutadiene resin and heated to 135° C. for 3 hours thereby to form a hardened layer of the resin in all the layers of the coil assembly. Then, a silicone rubber corona tire was placed on the surface of the deposited resin layer in the ordinary manner thereby to prepare a high-voltage coil.

The high-voltage coils prepared in examples 1 and 2 were incorporated into a flyback transformer in the ordinary manner, and various tests for determining the characteristics of the present high-voltage coils were conducted by incorporating the thus prepared flyback transformer into a television set. For comparison purpose, the conventional high-voltage coil for the flyback transformer was prepared according to the following manner and tested at the same time.

## Preparation of the conventional high-voltage coil:

A coil was prepared by winding a 0.12 Φ polyurethane-insulated wire using a 0.08 mm.-thick kraft paper tape as an interlayer insulating material. Then, the wound assembly was impregnated with microcrystalline wax, and an adhesive was applied onto the side surface of the thus impregnated coil. Finally, the corona tire was placed on the surface of the coil in the ordinary manner thereby to prepare a high voltage coil.

## 1. Temperature rise test:

The flyback transformers were mounted on television sets, and the tests were conducted at an ambient temperature of 40° C. The results are given in the following table.

|                                | Sample No. | Temperature rise<br>(°C.) |
|--------------------------------|------------|---------------------------|
| Conventional Coil              | 1          | 75.5                      |
|                                | 2          | 79.0                      |
| Coil according to<br>Example 1 | 1          | 69.2                      |
|                                | 2          | 62.9                      |
| Coil according to<br>Example 2 | 1          | 60.4                      |
|                                | 2          | 57.4                      |

## 2. Reduced pressure test:

Test (A): Insulating effects between the high pressure coil and core, and between coil layers of the flyback transformer were compared in a reduced pressure state. The testing procedure was such that the flyback transformer was placed in a pressure-reducible, closed vessel; the inside pressure was gradually reduced; and the atmospheric pressure at spark was measured (high voltage output : 27 kv.). The results are given in the following table.

|                             | Sample No. | Flyback transformer left at ordinary temperature | Flyback transformer left at 100° C. for 1 hour |
|-----------------------------|------------|--------------------------------------------------|------------------------------------------------|
| Conventional coil           | 1          | 365 mm. hg.                                      | 420 mm. hg.                                    |
|                             | 2          | 385                                              | 420                                            |
| Coil according to Example 1 | 1          | 380                                              | 420                                            |
|                             | 2          | 330                                              | 420                                            |
| Coil according to Example 2 | 1          | 385                                              | 420                                            |
|                             | 2          | 360                                              | 420                                            |

## Test (B):

Core used in the test (A) was replaced with a larger core and the pressure-withstanding time was measured (transformers left at the ordinary temperature were used).

The results are given in the following table.

|    | Sample No.                  | Result                                                                                                                 |
|----|-----------------------------|------------------------------------------------------------------------------------------------------------------------|
| 5  | 1                           | No high-voltage output was obtained at 350 mm. Hg for 20 seconds, and burning took place at 320 mm. Hg after 4 minutes |
|    | 2                           | Sparks were observed between a high-voltage coil heater and bobbin at 350 mm. Hg and test failed to continue           |
| 10 | Coil according to example 1 | No abnormal state was observed at 350 mm. Hg for 30 minutes                                                            |
|    | Coil according to example 2 | Same as above                                                                                                          |
|    |                             |                                                                                                                        |

## 3. Ozone-withstanding test:

Since the output voltage of flyback transformer is high, ozone is generated during the working. Thus, the ozone resistances of the impregnating agent were compared. Test pieces having a diameter of 50 mm. and thickness of 5 mm. were prepared from microcrystalline wax and 1-2 polybutadiene resin respectively, and were left in an atmosphere having an ozone concentration of 50 to 57 p.p.m. (50 to 57 cc. of ozone in one cubic centimeter) at a temperature of 40±1° C. for 10 hours. The results are given in the following table.

|                                     | Result                                        |
|-------------------------------------|-----------------------------------------------|
| Conventional (Microcrystalline wax) | Cracks were developed in the wax test piece   |
| 1-2 Polybutadiene                   | No abnormal state such as cracks was observed |

## 4. Boiling test:

Boiling test of the high-voltage coils was conducted to compare water-resistance of coils. Coils were boiled for 1 hour and 30 minutes, washed with water for 30 minutes, and left in air for 1 hour and then aged. The results are given in the following table

|                                  | Output                   |                       |                       |
|----------------------------------|--------------------------|-----------------------|-----------------------|
|                                  | Just after mounting (KV) | After 10 minutes (KV) | After 15 minutes (KV) |
| Conventional coil.....           | 1                        | 0                     | 5                     |
|                                  | 2                        | 5                     | 5.5                   |
| Coil according to Example 1..... | 1                        | 25.5                  | 25.5                  |
|                                  | 2                        | 23.0                  | 23.0                  |

55

## 5. Life test:

Flyback transformers incorporating a high-voltage coils prepared according to examples were mounted on television sets, and an 500-hour continuous test was conducted at an overload condition to check the life of the coil, but no abnormal states were observed. The ambient temperature was 41° to 43° C.

As is clear from the result of the foregoing tests, the present coil is excellent in water-resistance, moisture resistance, insulating efficiency, etc., and since the resin having a less dielectric loss at both low and high temperatures, for example, 20°-150° C., is used as an impregnating material, the temperature rise of the flyback transformer is so low that no burning of coil takes place.

Further, as the heat-setting impregnating resin is used, there is no disadvantage of fluidization as seen in the conventional wax, and the coil is not deformed even by application of heat and pressure thereto when a corona tire is placed thereon.

75 Thus, a coil having a uniform and high quality can be

prepared. Furthermore, impregnation, baking or other working can be readily conducted in preparing a coil.

As stated above, the present coil has various distinguished effects and utility over the conventional coil.

1. A coil for flyback transformer for television receiver, which comprises surface-insulated wire windings in a coil form having a plurality of wire layers, a plurality of layers of insulating material, adjacent layers of wound wires being separated by a layer of said insulating material, a corona tire attached to said coil, and an assembly of the wirings and interpositioned insulating material being impregnated with a resin consisting essentially of a polybutadiene in which said polybutadiene consists essentially of 1, 2 polybutadiene having a specific gravity of about 0.86 to about 0.90 and a mean molecular 15

weight of about 1,000 to about 5,000 said resin being heat hardened and having a low dielectric loss factor at both 20° C. and 150° C and a shore D hardness between 64 and 75 in said heat hardened form, said resin having been applied in a liquid form.

2. A coil according to claim 1 wherein said heat hardened resin has a density (g./cm.<sup>3</sup>) between about 0.94 and about 0.97, a bending strength (kg./mm.<sup>2</sup>) between about 3.0 and about 3.5 (ASTM-D-790), a compression strength (kg./mm.<sup>2</sup>) between about 7.1 and about 8.6.

3. A coil according to claim 1 wherein said insulating material is a kraft paper tape or polyethylene terephthalate tape.

\* \* \* \* \*

20

25

30

35

40

45

50

55

60

65

70

75